

## United States Patent [19]

Brown

[11] Patent Number: 4,610,101

[45] Date of Patent: Sep. 9, 1986

## [54] ORTHOTIC INSERT

[75] Inventor: Dennis N. Brown, Custer, Wash.  
 [73] Assignee: Northwest Podiatric Laboratories, Inc., Blaine, Wash.

[21] Appl. No.: 719,341

[22] Filed: Apr. 3, 1985

[51] Int. Cl.<sup>4</sup> ..... A43B 13/38[52] U.S. Cl. ..... 36/44; 36/76 C;  
 36/80; 12/146 M; 12/146 S; 128/614; 428/408[58] Field of Search ..... 36/44, 43, 76 C, 22 A;  
 12/146 M, 146 S, 146 R, 142 N; 428/408;  
 128/581, 586, 595, 614, 615

## [56] References Cited

## U.S. PATENT DOCUMENTS

2,644,250 7/1953 Ciaio ..... 36/76 C  
 4,023,801 5/1977 Van Auken ..... 428/408 X  
 4,186,499 2/1980 Massok, Jr. et al. ..... 36/44  
 4,231,169 11/1980 Toyama et al. ..... 36/44 X

4,338,734 7/1982 Schwartz ..... 36/44  
 4,368,234 1/1983 Palmer et al. ..... 428/408 X  
 4,439,934 4/1984 Brown ..... 36/44  
 4,520,581 6/1985 Irwin et al. ..... 36/44 X

## OTHER PUBLICATIONS

*The Runner*, Nov. 1982, Paying Through the Feet by Hal Higdon, pp. 86, 87, 88, 89 and 90.

Primary Examiner—James Kee Chi  
 Attorney, Agent, or Firm—Hughes & Cassidy

[57]

## ABSTRACT

An orthotic insert formed of a plurality of layers bonded to one another. Some of the layers are made from fiberglass reinforced plastic, having the fibers oriented at 45° from the longitudinal axis. At least one of the layers is made of parallel graphite fibers, having an axis of orientation offset from the longitudinal axis of the insert.

8 Claims, 16 Drawing Figures



FIG. 1



FIG. 2



FIG. 3



FIG. 4a



FIG. 4b



FIG. 5a



FIG. 5b

FIG. 6a

FIG.  
6b

FIG. 7A



FIG. 8



FIG. 9



FIG. 10



FIG. 7b



FIG. 11



FIG. 12



## ORTHOTIC INSERT

## CROSS REFERENCE TO RELATED APPLICATIONS

The subject matter of the present invention is related to the subject matter of five related patent applications being filed concurrently by the same applicant as in the present application, these five related applications being entitled: "Reinforced Heel Orthotic Insert", Ser. No. 719,324; "Orthotic For Athletic Use", Ser. No. 719,347; "Orthotic Insert for High Heeled Shoes", Ser. No. 719,348; "Reinforced Orthotic Insert", Ser. No. 719,413; and "Improved Orthotic for Running", Ser. No. 719,479.

The subject matter of these five related applications is hereby incorporated by reference to the same.

## BACKGROUND OF THE INVENTION

## 1. Field of the Invention

The present invention relates to an orthotic insert, and more particularly for such an insert which is particularly adapted to function effective throughout the gait cycle experienced in the common walking motion and in the common jogging motion.

## 2. Background Art

An orthotic insert can be either soft or hard. A hard insert is a substantially rigid member, desirably having a relatively thin vertical thickness dimension and extending from the calcaneus area of the foot (the heel portion) to at least the metatarsal head area of the foot (i.e. that area at the "ball" of the foot). In general, the purpose of a rigid orthotic (sometimes called a functional orthotic) is to first position, and then to control the movements of, the midtarsal and subtalar joints during the gait cycle which the body goes through in walking and running, and also possibly for other movements.

It is believed that a clearer understanding of the background of the present invention will be achieved by first discussing generally: (a) the main components or parts of the human leg and foot and how these function relative to one another; (b) the gait cycle which a person goes through in a normal walking motion; and (c) the intended function of a rigid orthotic in optimizing the coordinated operation of the person's foot and leg throughout the gait cycle.

For convenience, these various topics will be discussed under appropriate subheadings.

## (a) The Main Components or Parts of the Human Leg and Foot and How These Function Relative to One Another

With reference to FIGS. 1-3, there is shown a typical human foot 10, and (in FIGS. 2 and 3) the lower part 12 of the leg 14. The two lower bones of the leg 14 are the tibia 16 and the fibula 18. Below the tibia 16 and fibula 18, there is the talus 20 (i.e. the "ankle bone"). Positioned below and rearwardly of the talus 20 is the calcaneus 22 (i.e. the heel bone). Positioned moderately below and forward of the talus 20 are the navicular 24 and the cuboid 26. Extending forwardly from the navicular 24 are the three cuneiform bones 28. Extending forwardly from the cuneiform bones 28 and form the cuboid 26 are the five metatarsals 30. Forwardly of the metatarsals 30 are the phalanges 32 which make up the five toes 34.

The movement of the talus 20 relative to the tibia 16 and fibula 18 is such that it enables the entire foot to be

articulated upwardly and downwardly (in the motion of raising or lowering the forward part of the foot). However, the talus 20 is connected to the tibia 16 and fibula 18 in such a way that when the entire leg 14 rotated about its vertical axis (i.e. the axis extending the length of the leg), the talus 20 rotates with the leg 14.

With regard to the relationship of the talus 20 to the calcaneus 22, these move relative to one another about what is called the "subtalar joint" indicated at 36. The subtalar joint 36 can be described generally as a hinge joint about which the talus 20 and calcaneus 22 articulate relative to one another. The hinge axis extends upwardly and forwardly at an angle of about 42° from the horizontal, and also slants forwardly and inwardly at a moderate angle (e.g. about 16° from a straightforward direction). There is also the midtarsal joint 38, and this will be discussed later.

To explain further the hinge motion of the subtalar joint 36, reference is now made to FIGS. 4a and 4b. The talus 20 can be considered as a vertical board 40, and the calcaneus 22 as a horizontally extending board 42, these being hinge connected to one another along a diagonal hinge line 44, with this hinge line corresponding to the subtalar joint 36. It can be seen with reference to FIG. 4a that as the talus 20 is rotated inwardly about its vertical axis (i.e. the front part of the leg being rotated toward the center of the person's body), there is a corresponding rotation of the calcaneus 22 (i.e. the horizontal board 42) about a horizontal axis. It can be seen in FIG. 4b that an opposite (i.e. outward) rotation of the talus 20 (i.e. the vertical board 40) causes a corresponding rotation of the calcaneus 22 (i.e. the horizontal board 42) in the opposite direction to that shown in FIG. 4a.

This motion described with reference to FIGS. 4a and 4b above is critical in the gait cycle (i.e. the cycle through which the person goes in normal walking or running motion), and this will be discussed more fully below.

With regard to the midtarsal joint 38, this is in reality composed of two separate joints, the talo-navicular and the calcaneal-cuboid. It is a complex joint, and no attempt will be made to illustrate or recreate its motion accurately. Instead, there will be presented a somewhat simplified explanation of its function as it relates to the present invention.

The main concern, relative to the midtarsal joint, is not the precise relative motion of the parts of the foot that make up this joint, but rather the locking and unlocking mechanism of the midtarsal joint which occurs when there is an outward motion of the leg 14 and the talus 20 (outward motion meaning the rotation of the leg 14 about the vertical axis of the leg 14 in a manner that the knee moves outwardly from the person's body), and an opposite inward motion, respectively. When the leg 14 rotates inwardly, the midtarsal joint 38 unlocks so that the portion of the foot 10 forwardly of the joint 38 (i.e. the midfoot 45) is flexible, this being the "pronated" position of the foot. On the other hand, when the leg 14 and talus 20 rotate outwardly, the foot is said to be "supinated" so that the midtarsal joint 38 is locked and the midfoot 45 essentially becomes a part of a rigid lever. In actuality, the midfoot 45 never becomes totally rigid, so that even in the totally supinated position, there is some degree of flexibility in the midfoot 45.

This function of the midtarsal joint will now be explained relative to FIGS. 5a and 5b. It can be seen that FIGS. 5a-b are generally the same as FIGS. 4a-b, ex-

cept that a forward board member 46 is shown to represent the midfoot 45, this member 46 having a downward taper in a forward direction, and also a lower horizontal plate portion 48. This plate portion 48 is intended to represent that the plantar surface (i.e. the lower support surface) of the midfoot 45 engages the underlying support surface in a manner so as to remain generally horizontal to the support surface.

It can be seen that when the two board members 40 and 42 are in the pronated position of FIG. 5a, the 10 metatarsal joint represented at 50 in FIGS. 5a-b is in a first position which will be presumed to be an unlocked position. In the unlocked position of FIG. 5a, the member 46 is not rigid with the horizontal member 42, and the forward member 46 can flex upwardly relative to 15 the horizontal member 42. (This is the pronated position of the foot 10). However, in the position of FIG. 5b, the board members 46 and 42 will be presumed to be locked to one another so that the members 42 and 46 form a unitary lever. For ease of illustration, no attempt has 20 been made to illustrate physically the unlocking relationship of FIG. 5a and the locking relationship of FIG. 5b. Rather, the illustrations of FIGS. 5a-b are to show the relative movement of these components, and the locking and unlocking mechanism is presumed to exist. 25

(b) The Gate Cycle Which the Person Goes Through in a Normal Walking Motion

Reference is first made to FIGS. 6a and 6b. As illustrated in the graph of FIG. 6a, during the normal walking motion, the hip (i.e. the pelvis) moves on a transverse plane, and this movement in the gait cycle is illustrated in FIG. 6b. Also, the femur (i.e. the leg bone between the knee joint and the hip) and the tibia rotate about an axis parallel to the length of the person's leg. (It is this rotation of the leg about its vertical axis which in large part causes the pronating and supinating of the foot during the gait cycle, and this will be explained in more detail below.)

There is also the flexing and extension of the knee, as 40 illustrated in the five figures immediately below the graph of FIG. 6a. Further, there is the flexing and gait cycle, the heel of the forwardly positioned leg strikes the ground, after which the forward part of the foot rotates downwardly into ground engagement. After the 45 leg continues through its walking motion to extend rearwardly during the gait cycle, the person pushes off from the ball of the foot as the other leg comes into ground engagement.

The motions described above are in large part generally apparent to a relatively casual observation of a person walking. However, the motion which is generally overlooked by those not familiar with the gait cycle is the inward and outward rotation of the leg about its lengthwise axis to cause the pronating and supinating of 55 the foot through the gait cycle. This will be described relative to FIG. 7a and FIG. 7b.

When the leg is swung forwardly and makes initial ground contact, at the moment of ground contact the leg is rotated moderately to the outside (i.e. the knee of the leg is at a more outward position away from the centerline of the body) so that the foot is more toward the supinated position (i.e. closer to the position shown in FIG. 4b). However, as the person moves further through the gait cycle toward the 25% position shown in FIG. 7a, the leg rotates about its vertical axis in an inside direction so that the subtalar joint is pronating. The effect of this is to rotate the heel of the foot so that

the point of pressure or contact moves from an outside rear heel location (shown at 52 in FIG. 7b) toward a location indicated at 54 in FIG. 7b. This pronating of the subtalar joint 36 produces a degree of relaxation of the midtarsal joint 38 and subsequent relaxation of the other stabilization mechanisms within the arch of the foot. This reduces the potential shock that would otherwise be imparted to the foot by the forward part of the foot making ground contact.

With further movement from the 25% to the 75% position, the leg rotates in an opposite direction (i.e., to the outside so that the midtarsal joint 38 becomes supinated at the 75% location of FIG. 7a. This locks the midtarsal joint 38 so that the person is then able to operate his or her foot as a rigid lever so as to raise up onto the ball of the foot and push off as the other leg moves into ground contact at a more forward location.

With reference again to FIG. 7b, the initial pressure at ground contact is at 52 and moves laterally across the heel to the location at 54. Thereafter, the pressure center moves rather quickly along the broken line indicated at 56 toward the ball of the foot. As the person pushes off from the ball of the foot and then to some extent from the toes of the foot, the center of pressure moves to the location at 58.

(c) The Intended Function of the Orthotic to Improve Operation of the Person's Foot and Leg Throughout the Gate Cycle

If the person's foot were perfectly formed, then there would be no need for an orthotic device. However, the feet of most people deviate from the ideal. Accordingly, the function of the orthotic is first to position the plantar surface of the calcaneus 22 and the midfoot 45 so that the subtalar and midtarsal joints 36 and 38 are initially positioned properly (i.e., to bring the person's foot back to the ideal functioning position peculiar to the person's foot), and to thus control the subsequent motion of the foot parts or components that make up these joints so that the movements of the hip, leg and foot throughout the gait cycle are properly accomplished. It can be readily understood that if the components of the foot have the proper initial position and movement about the subtalar and midtarsal joints 36 and 38, the entire gait cycle, all the way from the coordinated rotation of the hips through the flexing and rotation of the leg, and also through the initial strike of the heel on the ground to the final push off from the toe of the foot, is properly coordinated and balanced for optimum movement.

Since shoes are generally manufactured on a mass production basis, the supporting surface of the interior of the shoe may or may not optimally locate the plantar surface of the foot. Accordingly, it has for many years been a practice to provide an orthotic insert which fits within the shoe to optimize the locations of the foot components. In general, these inserts have been made of various materials, some of which are formed as laminated structures to provide a relatively rigid support for the heel and midfoot regions of the foot.

These orthotics can be formed in a variety of ways. A preferred method of forming an orthotic insert is described in the applicant's U.S. Pat. No. 3,995,002. In that method, there is formed a negative mold or slipper cast from which a positive cast of the plantar surface of the individual's foot is formed. Using this positive cast as a template, an orthotic insert is formed to underlie an area under the foot. The insert itself is fabricated by applying to the positive cast the material which is to be

the orthotic insert. The precise configuration of the insert will depend upon the prescribed corrective measures to be taken for the individual's foot.

#### SUMMARY OF THE INVENTION

The present invention embodies the broad teachings of U.S. Pat. No. 4,439,934, and provides specific improvements for the same.

There is a substantial unitary orthotic insert adapted to be placed in an article of footwear. The insert has a longitudinal axis parallel to a lengthwise axis of a foot for which the insert is used, and a transverse axis.

The insert comprises a rear portion adapted to underlie and engage a plantar surface of a calcaneal area of the foot. There is a forward portion adapted to underlie and engage a plantar surface of a metatarsal head area of the foot. There is an intermediate portion connecting to and extending between said rear and forward portions to engage a plantar surface of a mid-foot area of the foot.

The insert has outside and inside edge portions adapted to be engaged and adjacent an outside edge and an inside edge of the foot, respectively.

The insert has a laminated structure comprising a plurality of vertically stacked layers bonded to one another to form a substantially unitary structure. The laminated structure comprises a first laminate means having an internal material structure adapted to resist bending moments generally uniformly about both its said longitudinal and transverse axes.

There is a second laminate means comprising a layer having fibers which have a predominate orientation of alignment about a direction extending from a rear outside location to a forward inside location, so as to provide greater resistance to bending moments along a first axis extending from a rear outside location to a forward inside location generally parallel to said orientation, and to provide less resistance to bending along a second axis extending from a rear inside portion to forward outside portion generally perpendicular to said orientation.

The laminated structure is characterized in that the structure has an overall greater resistance to bending along the first axis, relative to the second axis.

In the preferred form, the fibers of the second laminate means are positioned relative to the longitudinal axis at an angle greater than zero degrees to the longitudinal axis, and an angle no greater than about 45° to the longitudinal axis. In the preferred embodiment, the fibers of the second laminate means are at an angle to the longitudinal axis of approximately one-third of a right angle.

Desirably, the second laminate means comprises at least one layer having a plurality of graphite fibers having said predominate orientation. Also in the preferred embodiment, the first laminate means comprises at least one layer having fibers oriented at generally right angles to one another in a manner to provide more uniform bending resistance about both longitudinal and transverse axes.

More desirably, the first laminate means comprises a plurality of layers, with each of the layers having fibers oriented with respect to one another at generally right angles. These are arranged so as to provide more uniform resistance to bending along both longitudinal and transverse axes.

In a specific embodiment, a forward inside portion of said first laminate means is removed, thereby creating greater resistance to bending at the rear portion and at the outside edge portion of the foot.

With regard to specific materials, in the preferred embodiment, the first laminate means comprises a plurality of layers of fiberglass impregnated with resin. The second laminate means comprises at least one layer of graphite fibers.

Other features of the present invention will become apparent from the following detailed description.

#### BRIEF DESCRIPTION OF THE DRAWINGS

FIG. 1 is a top plan view of the right foot of a human, with certain components of the foot being separated from one another for purposes of illustration;

FIG. 2 is a side elevation view looking toward the inside of a person's left foot, with the outline of the foot and lower leg being shown as a shaded area;

FIG. 3 is a view similar to FIG. 2, but looking toward the outside of the person's foot;

FIGS. 4a and 4b are perspective views illustrating schematically the rotational movements of the talus and calcaneus about the subtalar joint;

FIGS. 5a and 5b are schematic views similar to those of FIGS. 4a-b, but further illustrating the relative movement between the calcaneus and the midfoot about the midtarsal joint;

FIG. 6a is a graph illustrating the rotational movement of the pelvis, femur and tibia during one-half of a gait cycle;

FIG. 6b is a top plan view illustrating the rotation of the person's pelvis during that portion of the gait cycle illustrated in FIG. 7a;

FIG. 7a is a graph similar to FIG. 6a, but illustrating the timing of the pronating and supinating motion of the leg and foot through one-half of a gait cycle;

FIG. 7b is a view looking upwardly toward the plantar surface of a person's left foot, and illustrating the distribution of location of the center of pressure throughout the period of ground contact of the portion of the gait cycle illustrated in FIGS. 6a and 7a;

FIG. 8 is a top plan view of an upper soft portion of an orthotic device, made to fit a person's right foot;

FIG. 9 is a top plan view of another portion of the orthotic insert toward which the subject matter of the present invention is particularly directed;

FIG. 10 is an isometric view of an insert made in accordance with the present invention;

FIG. 11 is a perspective view of six laminations utilized in forming the first embodiment of the present invention to form the insert section illustrated in FIG. 9; and

FIG. 12 is a view similar to FIG. 11, showing the laminations to form a second embodiment of the present invention which is another form of the insert section illustrated in FIG. 9.

#### DESCRIPTION OF THE PREFERRED EMBODIMENTS

The present invention comprises a more specific improvement of the orthotic insert described in the applicant's issued U.S. Pat. No. 4,439,934.

As described in that patent, the overall method for forming the insert is generally the same as that described in applicant's U.S. Pat. No. 3,995,002. There is first provided a negative mold, from which a positive cast (i.e. a cast resembling the structure of a person's foot) is formed. Using this positive cast as a template, an orthotic insert is formed to underlie the structure of a person's foot) is formed. Using this positive cast as a template, an orthotic insert is formed to underlie the

area of the foot from the calcaneal area forward to the first metatarsal head, including the arch area, and from there laterally to the distal side of the foot or fifth metatarsal head. The insert itself is fabricated by applying to the positive cast layers of fiber impregnated with resin. The assembled layers are then heat cured and cut to the limits of the cast.

As further discussed in the applicant's U.S. Pat. No. 4,439,934, the flexing characteristics of the insert, which are integral to its performance, can be beneficially controlled by adjusting the placement, amount and direction of graphite fibers, and in some instances, other fibers such as glass fibers. The insert so formed is extremely light weight and relative thin in comparison to conventional orthotic inserts.

To proceed to a more detailed description of the present invention, in FIG. 8, there is shown a two layered first blank 60 which is generally configured to the outline of a bottom of an individual's foot. This blank 60 can be of conventional configuration. For example, it can include an upper layer of a cloth material such as nylon, Dacron, cotton or the like which is abrasion resistant and absorbs perspiration well. It can further comprise a second layer of flexible rubber or neoprene or the like which is co-extensive with and adheres to the upper layer. While this first blank 60 is desirably used in the present invention, within the broader aspects of the present invention, this blank 60 is not an absolutely necessary element.

In FIG. 9, there is a second blank 62 which incorporates the teachings of the present invention. In the end configuration of the present invention, this blank 62 underlies the blank 60 and is bonded thereto. The end configuration of the two blanks 60 and 62 is illustrated in FIG. 10, which is a perspective view of the end product indicated at 64.

In the applicant's earlier patent, U.S. Pat. No. 4,439,934, the method of forming the blank 62 was described generally. This blank 62 can be formed and contoured around a positive cast obtained using the method and apparatus disclosed in applicant's U.S. Pat. No. 3,995,002, or by some other method. Then various arrangements of layers of fiberglass or graphite, impregnated with resin, are laid upon the positive cast to form the second blank 62.

With respect to the novel features of the present invention, it has been found that within the broad teaching of U.S. Pat. No. 4,439,934, the orientation of certain of the fibers in the layer or layers can be selected in certain configuration to improve the performance characteristics of the orthotic insert in specific ways.

FIG. 11 illustrates a first embodiment of the present invention, and it can be seen that this is made up of six layers, designated 70a-f, each having the general shape of the blank 62 illustrated in FIG. 9. Five of the layers (70a-d and f) are identical, and each comprises a fiberglass resin layer, where the fiberglass strands are arranged in a right angle crossing pattern. The fiberglass layer is cut so that in the end configuration, the two sets of strands are at a 45° angle to the lengthwise or longitudinal axis 72 of the insert. Thus, the overall resistance to bending imparted by these five layers (i.e. 70a-d and f) is generally uniform for a given thickness over the face of the insert. A fiberglass resin laminate suitable for use as these inserts is designated as 7781, manufactured by Hexcel.

The layer 70e is made up of a plurality of graphite strands, all oriented parallel to each other, with these

5 being impregnated with a suitable resin. It will be noted that in the embodiment shown herein, the strands of the graphite in the layer 70e extend in a diagonal line from a rear outside portion of the insert toward a forward inside portion of the insert. As shown herein, the graphite strands are desirably oriented at 30° off the horizontal axis. In the preferred form, however, this precise orientation can vary depending upon the particular function to be accomplished. In general, the orientation of these strands indicated by the line 74 relative to the longitudinal axis 72 would be greater than 0° from the longitudinal axis 72, and generally no greater than about one-half of a right angle from the longitudinal axis 72.

10 The layers 70a-f are bonded and cured to form the unitary blank 62. More specifically, the layers 70a-f can be conformed to the contour of the mold, preheated for a period of time, cured at, for example, 350° F. for about 45 minutes, and then be affixed to the bottom of the first blank 60 to create the final insert 64.

15 In operation, the laminates 70a-f, being bonded to one another in a unitary structure, have greatest resistance to bending along the axis (indicated at 74) parallel to the orientation of the graphite strands of layer 70e. The blank 62 has the least resistance to bending along a second axis 76 which is perpendicular to the alignment axis 74. Thus, the greatest resistance to bending is relative to forces transmitted perpendicular to the blank 62 at spaced locations along an axis extending from the forward inside portion of the insert 62 to the rear outside portion thereof. The least resistance to bending is along the axis 76 from an inside portion of the insert toward the outside edge thereof.

20 With regard to the results achieved by the present invention, it should be appreciated that during the gait cycle, the application of the force of the foot to the underlying ground surface is not totally uniform. Usually, there is an abrupt increase in the force applied as the heel comes into ground engagement. This is followed by a moderate increase in force as the foot proceeds through the gait cycle. During the final portion of the gait cycle, the person is pushing off from the inside portion of the ball of the foot and from the big toe. This arrangement of the insert is uniquely arranged to accomplish proper support during that cycle.

25 A second embodiment of the present invention is illustrated in FIG. 12. In this particular embodiment, there are eight layers 80a-h. The first and third layers 80a and 80c are made from a fiberglass resin sheet, such as those of the first embodiment (i.e. sheets 70a-d and 70f). The second layer 80b is formed from a graphite impregnated sheet, with the layer cut so that the orientation of the graphite fibers is at 30° to the lengthwise axis 82. The fourth, fifth and sixth layers, 80d-f are also made or cut from a graphite fiber/resin sheet, with the orientation of the graphite fibers being directly parallel to the longitudinal axis.

30 The seventh layer 80g is cut from a fiberglass resin sheet, but the orientation of the glass fibers are parallel to the longitudinal axis and perpendicular thereto. Finally, the lowermost layer 80h is made as a graphite/resin layer, with the orientation of the fibers also being at 30° from the longitudinal axis, and directed in a forward and inside direction.

35 Further, the middle and forward inside edge portions, indicated at 84g and 84h, of layers 80g and 80h are cut away, so that the heel portion and outside portions of the blank 62 are strengthened relative to the cut out portions 84g-h.

It has been found that the arrangement of this second embodiment shown in FIG. 12 is particularly advantageous in supporting a person's foot during normal straight ahead running, such as in jogging. Analysis has shown that the instantaneous forces applied to a normal jogger's foot can be very abrupt, and much greater than in walking. For example, for a person having a body weight of 160 pounds, the instantaneous force on the foot during jogging at a moderate pace can rise to a level of nearly 400 pounds or possibly greater. Also, there is a rather abrupt and sharp force applied to the heel of the foot at the moment of impact of the heel to the ground surface.

It has been found that the inward and forward orientation of some of the graphite fibers provide the same beneficial resistance to bending along that axis, as in the first embodiment of FIG. 11. However, in addition, the present invention, with the orientation of the graphite fibers of three of the layers (i.e.  $80d-f$ ) being directly longitudinal, there is substantial resistance to bending along the lengthwise axis of the insert. However, there is less resistance to bending transverse to the longitudinal axis, and this permits the moderate flexibility along an axis where greater resistance to bending is not required.

It is to be understood that within the broader scope of the embodiments shown herein, the angular variation of the fibers can be modified, depending upon the special requirements of the person's foot. Also, while the particular layup of these layers has been found to be quite advantageous, it is to be understood that certain additions or deletions could be made depending upon the particular circumstances relating to that person's foot. Also, the order or placement of the layers could be modified and still function within the general mode of operation of the present invention.

What is claimed is:

1. A substantially unitary orthotic insert adapted to be placed in an article of footwear, said insert having a longitudinal axis parallel to a lengthwise axis of a foot 40 for which the insert is used, and a transverse axis, said insert comprising:
  - a. a rear portion adapted to underlie and engage a plantar surface of a calcaneal area of the foot;
  - b. a forward portion adapted to underlie and engage 45 a plantar surface of a metatarsal head area of the foot;
  - c. an intermediate portion connecting to and extending between said rear and forward portions to engage a plantar surface of a mid-foot area of the foot;
  - d. said insert having outside and inside edge portions 50 adapted to be positioned adjacent an outside edge and an inside edge of the foot, respectively;
  - e. said insert having a laminated structure comprising a plurality of vertically stacked layers bonded to one another to form a substantially unitary structure, said laminated structure comprising:
    1. first laminate means having an internal material structure adapted to resist bending moments generally uniformly about both of said longitudinal and transverse axes;

2. a second laminate means comprising a layer having fibers which have a predominant orientation of alignment about a direction extending from a rear outside location to a forward inside location, so as to provide greater resistance to bending moments along a first axis extending from a rear outside location to a forward inside location generally parallel to said orientation, and to provide less resistance to bending along a second axis extending from a rear inside portion to a forward outside portion generally perpendicular to said orientation;
- f. said laminated structure being characterized in that said structure has an overall greater resistance to bending along said first axis, relative to said second axis.
2. The insert as recited in claim 1, wherein the fibers of said second laminate means are positioned relative to said longitudinal axis at an angle greater than  $0^\circ$  to said longitudinal axis, and at an angle no greater than about  $45^\circ$  to said longitudinal axis.
3. The insert as recited in claim 2, wherein the fibers of said second laminate means are at an angle to the longitudinal axis of approximately one-third of a right angle.
4. The insert as recited in any of claims 1, 2 or 3, wherein said second laminate means comprises at least one layer having a plurality of graphite fibers having said predominant orientation.
5. The insert as recited in any of claims 1, 2 or 3, wherein the fibers of said second laminate means comprise graphite fibers having said predominant orientation, and said first laminate means comprising at least one layer having fibers oriented at generally right angles to one another in a manner to provide more uniform bending resistance about both longitudinal and transverse axes.
6. The insert as recited in any one of claims 1, 2 or 3, wherein there is a plurality of layers comprising said first laminate means, each of the layers in said plurality having fibers oriented with respect to one another at generally right angles, and arranged so as to provide more uniform resistance to bending along both longitudinal and transverse axes.
7. The insert as recited in any one of claims 1, 2 or 3, wherein at least one layer of one of said first laminate means has an inside forward portion thereof removed, thereby creating greater resistance to bending at the rear portion and at the outside edge portion of the foot.
8. The insert as recited in any one of claims 1, 2 or 3, wherein said first laminate means comprises a plurality of layers of fiberglass impregnated with resin, with orientation of said fiberglass being along two axes at right angles to one another, with the orientation being generally at a half of a right angle to the longitudinal axis of the insert, said second laminate means comprising at least one layer graphite fibers having the orientation of the second laminate means being at approximately a third of a right angle from the longitudinal axis.

\* \* \* \* \*